

# United States Patent

De Long et al.

[15] 3,656,918  
[45] Apr. 18, 1972

[54] COMPOSITE WELDED FERROUS ARTICLE

[72] Inventors: William T. De Long; Paul T. Corcoran, both of West Manchester Township, York County, Pa.

[73] Assignee: Teledyne, Inc., Los Angeles, Calif.

[22] Filed: Dec. 30, 1969

[21] Appl. No.: 889,321

[52] U.S. Cl..... 29/196.1

[51] Int. Cl..... B32b 15/00

[58] Field of Search..... 29/196.1; 75/123 K, 128

[56] References Cited

## UNITED STATES PATENTS

|           |         |                  |          |
|-----------|---------|------------------|----------|
| 2,516,125 | 7/1950  | Kramer .....     | 75/123 K |
| 2,992,148 | 7/1961  | Yeo.....         | 75/123 K |
| 3,290,128 | 12/1960 | Manganello ..... | 75/128 V |

Primary Examiner—Hyland Bizot  
Attorney—Edward Hoopes, III

[57] ABSTRACT

A low carbon steel weld deposit containing chromium up to 1.0, preferably 0.05–0.6, per cent. by weight, nickel 6.5–11,

preferably 7–9, per cent. by weight, molybdenum up to 1.0, preferably 0.2–0.8, per cent. by weight and vanadium up to .12, preferably 0.04–0.09, per cent. by weight.

Also a low carbon steel weld deposit consisting essentially of

| Element         | Percent by Weight |           |
|-----------------|-------------------|-----------|
|                 | Broad             | Preferred |
| Carbon.....     | .03 – .12         | .06 – .10 |
| Manganese.....  | .05 – 1.0         | .1 – .8   |
| Silicon.....    | .20 – .70         | .25 – .55 |
| Chromium.....   | up to 1.10        | .05 – .6  |
| Nickel.....     | 6.5 – 11.         | 7 – 9     |
| Molybdenum..... | up to 1.0         | .2 – .8   |
| Vanadium.....   | up to .12         | .04 – .09 |
| Phosphorus..... | .020 max.         | .012 max. |
| Sulfur.....     | .020 max.         | .012 max. |
| Iron.....       | Balance           | Balance   |

which exhibits a yield strength of at least 130 ksi and Charpy V-notch energy absorption at –60° F. of at least 20 ft.-lbs. after heat treatment consisting of austenitizing at 1,500° F. for 1 hour, water quenching, tempering at 1,100° F. for 1 hour and water quenching.

1 Claim, No Drawings

## A COMPOSITE WELDED FERROUS ARTICLE

The invention herein described was made in the course of or under a contract or subcontract thereunder with the Department of the Navy.

This invention relates to steel weld deposits; more particularly, it relates to low alloy steel weld deposits which exhibit high strength and notch-toughness both as-welded and after heat treatment.

In the field of low alloy high strength steels with yield strengths above about 100 ksi, particularly HY-130/150 type steels with yield strengths of at least 130 ksi, there has been a need for high performance weld metals which in a single deposit will have yield and tensile strengths and impact toughness approximately equal to those of the base metal both as-deposited and in the heat treated (i.e., quenched and tempered) condition. Weld deposited metal is always under a handicap compared with plate material and must be more shrewdly formulated because it lacks the advantages of the mechanical hot work treatments which produce grain refinement in plate material. In spite of this handicap low alloy steel weld deposit analyses and methods of deposition have been developed which produce as-deposited metal with yield strength at least matching that of the available hot worked and heat treated plate material, coupled with suitable toughness. Requiring the highest quality welding processes, such deposits were recently produced by means of inert gas shielded methods used with high purity alloy-bearing filler wires. This level of performance has first been achieved with deposits from manual low hydrogen lime-fluoride covered electrodes, which was a more difficult goal. However, heat treatment of such deposits, often necessary in the fabrication of heavy sections, causes a drop in mechanical properties, often to levels which are unacceptable in the end use of the weldment.

We are able to produce steel weld deposits which exhibit yield strengths above 100 ksi and typically 130-160 ksi and Charpy V-notch toughness above 20 ft.-lbs. at -60° F. and typically 30-50 ft.-lbs. at -60° F., both as-deposited according to recommended procedures, and after a heat treatment typically consisting of austenitizing at 1,500° F. for 1 hour, water quenching, tempering at 1,100° F. for 1 hour and again water quenching. As compared to earlier weld metals of the HY-130/150 type, which are suitable for as-welded use but not for heat treatment, our weld deposits are characterized by a novel balance of those chemical elements which have proven most effective in the as-welded grades, and also by a retention of the earlier emphasis on limitations in the harmful elements phosphorus and sulfur to levels below 0.020 per cent. by weight and preferably below 0.012 per cent. by weight.

A particularly attractive aspect of our weld deposits is that they may exhibit the above mentioned as-deposited and heat-treated properties when deposited with low hydrogen lime-fluoride covered electrodes utilizing conventional commercial quality rimmed steel core wires. Such electrodes, which were the chosen means for producing weld deposits which established the existence and limitations of our invention, offer significant economic advantages over the simpler but much more expensive high purity wire and gas-metal-arc (GMA) processes which are also applicable and which have heretofore been widely used in investigating and producing HY-130/150 weld metals.

We provide low carbon steel weld deposits characterized by chromium up to 1.0 per cent. by weight, nickel 6.5 - 11 per cent. by weight, molybdenum up to 1.0 per cent. by weight and vanadium up to 0.12 per cent. by weight; the deposits preferably contain chromium 0.05 - 0.6 per cent. by weight, nickel 7 - 9 per cent. by weight, molybdenum 0.2 - 0.8 per cent. by weight and vanadium 0.04 - 0.09 per cent. by weight.

We further provide a weld deposit consisting essentially of

|           | Percent by Weight |
|-----------|-------------------|
| Carbon    | 0.03-0.12         |
| Manganese | 0.05-1.0          |
| Silicon   | 0.20-0.70         |

|            |            |
|------------|------------|
| Chromium   | up to 1.0  |
| Nickel     | 6.5-11     |
| Molybdenum | up to 1.0  |
| Vanadium   | up to 0.12 |
| Phosphorus | 0.020 max. |
| Sulfur     | 0.020 max. |
| Iron       | Balance    |

In a preferred form the deposit consists essentially of

|            | Percent by Weight |
|------------|-------------------|
| Carbon     | 0.06-0.10         |
| Manganese  | 0.1-0.8           |
| Silicon    | 0.25-0.55         |
| Chromium   | 0.05-0.6          |
| Nickel     | 7-9               |
| Molybdenum | 0.2-0.8           |
| Vanadium   | 0.04-0.09         |
| Phosphorus | 0.012 max.        |
| Sulfur     | 0.012 max.        |
| Iron       | Balance           |

20 We further provide such deposits that exhibit yield strengths of at least 130 ksi and Charpy V-notch energy absorption at -60° F. of at least 20 ft.-lbs. after heat treatment consisting of austenitizing at 1,500° F. for 1 hour, water quenching, tempering at 1,100° F. for 1 hour and water quenching.

25 Realization of the optimum as-welded properties of our improved weld deposits will depend on the conditions under which they are deposited, as will be appreciated by those skilled in the art. In the HY-130/150 area certain practices, such as low welding heat input and small bead size, are known

30 to maximize as-welded strength and toughness of the deposit; somewhat surprisingly, however, the as-welded properties of our deposits are relatively insensitive to heat input, which is a significant advantage when they are produced with covered electrodes under field conditions. In addition to such general

35 practices the specific welding process employed to produce our improved weld deposits will have a definite effect on the degree of retention of the maximum as-welded deposit properties attainable; it is well established that the higher the weld metal purity, the more its properties will approach the optimum for its overall alloy balance. "Purity" in this context not only means low levels of residual or tramp elements such as phosphorus, sulfur, nitrogen and oxygen but also includes aspects such as size and shape of inclusions, etc. The gas-tungsten-arc (GTA) process with pre-alloyed high purity filler

40 metal additions, which provides the highest purity weld metal, can be expected to be optimum for producing our deposits; somewhat lower on the scale, although still very good, is the GMA process utilizing argon-oxygen or equivalent shielding gases and pre-alloyed electrode wire. As above indicated, we

45 have also found that our new analysis can be weld deposited with good results close to those obtained with the GMA process and at much lower cost with properly formulated high quality low hydrogen lime-fluoride covered electrodes. Deposits produced by other types of covered electrodes or

50 submerged arc welding can be expected to exhibit inferior as-welded properties to a degree dependent on the specific process used and the purity of the resultant weld metal. Heat-treated properties are less dependent on welding processes and conditions since austenitizing of the deposit causes

55 recrystallization, which wipes out many of the effects of welding variables.

The low hydrogen lime-fluoride covered electrode which we have used for producing our deposits meets a general specification for this class of electrode and consists of a mild steel core and a lime-fluoride coating thereon, the electrode

60 containing by weight about 45 per cent. to about 80 per cent. core and about 20 per cent. to about 55 per cent. coating, the coating containing by weight of the electrode up to about 30 per cent. iron powder and alloying metal powder, about 2 per cent. to about 7 per cent. deoxidizer metal powder, about 4 per cent. to about 15 per cent. metal fluoride, about 5 per cent. to about 15 per cent. alkaline earth carbonate, 0 to about 10 per cent. slag builder and modifier and about 0.5 per cent. to about 8 per cent. inorganic binder material. Although

we have chosen to supply all alloy by way of the coating for reasons of economy in our electrode, it is of course possible to introduce all or part of the alloy through the core wire.

Other details, objects and advantages of the invention will become apparent as the following description of certain present preferred embodiments thereof proceeds.

TABLE 1  
Welding conditions used in preparing weld deposits 10  
A, B, C and D

Plate material: 2 pieces of one-inch-thick U.S. Steel HY-130(T) plate, minimum dimensions 10" long x 4" wide

Chemistry: 0.12% C, 0.90% Mn, 0.34% Si, 0.59% Cr, 4.96% Ni, 0.50% Mo, 0.064% V, 0.002% P, 0.008% S

Joint: Type—single V

Preparation—Flame cutting followed by grinding 20  
Bevel—22B° on each plate

Electrode:

Diameter—5/32"

Coating—Low hydrogen lime-fluoride type

Backup plate: U.S. Steel HY-130(T) one-inch-thick 25  
plate, one inch minimum in width x joint length

Welding position: Flat

Welding current: 185±5 amps DC, reverse polarity

Welding voltage: 24 volts

Heat input: 30±2 kilojoules per inch

Preheat and interpass temperature: 250° F.±25° F.

Interpass delay: 1 hour minimum

Core wire: Type—conventional commercial-quality  
rimmed steel

Chemistry—0.07% C, 0.50% Mn, 0.005% Si,  
0.007% P, 0.020% S

Table 2) with low hydrogen lime-fluoride covered electrodes. In preparing the deposits, only one welder and one power source were used, and all test weldments were made in the flat position using reverse polarity direct current. Multipass welds were prepared using stringer beads and a temper bead deposition sequence. Welding parameters were controlled so that a calculated heat input of  $30 \pm 2$  kilojoules per inch would be maintained. Each pass in a test weldment was completed with one electrode only and no starts or stops were located in the test area. Preheat and interpass temperatures of the test weldment were maintained at  $250^\circ \pm 25^\circ$  F. In an attempt to preclude any hydrogen-caused cracks in the deposit, a 1-hour minimum interpass delay time was used. Table 2 lists chemical compositions and mechanical test results obtained with the four deposits A, B, C and D after heat treatment in 1- and 4-inch-thick sections. Heat treatment consisted of austenitizing at  $1,500^\circ$  F. for 1 hour, water quenching, tempering at  $1,100^\circ$  F. for 1 hour and water quenching again; this cycle was simulated for the 4-inch thickness by blower cooling  $\frac{1}{2}$ -inch-thick sections from the austenitizing and the tempering temperatures. It will be seen that our deposits are not strongly affected by changes in manganese or nickel content within the above defined preferred limits; compare deposits A and B for example. Deposits A and B also illustrate that our preferred deposits show excellent heat-treated properties in section thicknesses as high as 4 inches. Chromium higher than our preferred limits but within our broad limits, as illustrated by deposits C and D, appears to lower the heat-treated yield strength in thick sections; for best performance we prefer chromium on the order of 0.5 per cent. Deposits C and D also illustrate the beneficial effect of small vanadium additions to our deposits. The two deposits are essentially equivalent except for vanadium content, and while both show decreases in heat-treated yield strength in thick sections because of chromium contents somewhat higher than optimum, it will be seen that the vanadium addition provides a significant increase in yield strength while causing only a relatively small loss in impact properties in view of the gain in yield strength.

TABLE 3  
Effect of heat input on as-welded properties  
Deposit E analysis: .085% C, .52% Mn, .51% Si, .43% Cr, 8.29% Ni, .49% Mo, .065% V

| Deposit | Heat input,<br>kilojoules<br>per inch | Yield<br>strength<br>(0.2%<br>offset),<br>K.s.i. |                      | Elong-<br>ation<br>in 2 inches,<br>percent |       | Reduction<br>of<br>area,<br>percent |      |      | Charpy V-notch energy<br>absorption, ft.-lb. |  |  |
|---------|---------------------------------------|--------------------------------------------------|----------------------|--------------------------------------------|-------|-------------------------------------|------|------|----------------------------------------------|--|--|
|         |                                       | Tensile<br>strength,<br>K.s.i.                   | 2 inches,<br>percent | 80° F.                                     | 0° F. | -60° F.                             |      |      |                                              |  |  |
| E       | 30.6                                  | 155                                              | 165                  | 16.4                                       | 59.9  | 47.8                                | 44.8 | 42.3 |                                              |  |  |
| F       | 59.3                                  | 145                                              | 167.5                | 15.7                                       | 54.8  | 46.8                                | 42.5 | 38.3 |                                              |  |  |

TABLE 2  
Compositions and properties of heat treated weld deposits

| Deposit | C    | Mn  | Si  | Cr  | Ni   | Mo  | V     | Plate<br>thick-<br>ness,<br>inches | Yield<br>strength<br>(0.2%<br>offset),<br>K.s.i. |                      | Elong-<br>ation<br>in 1.4<br>inches,<br>percent |       | Red. of<br>area,<br>percent | Charpy V-notch energy<br>absorption, ft.-lb. |       |         |
|---------|------|-----|-----|-----|------|-----|-------|------------------------------------|--------------------------------------------------|----------------------|-------------------------------------------------|-------|-----------------------------|----------------------------------------------|-------|---------|
|         |      |     |     |     |      |     |       |                                    | Tensile<br>strength,<br>K.s.i.                   | 2 inches,<br>percent | 80° F.                                          | 0° F. |                             | -80° F.                                      | 0° F. | -60° F. |
| A       | .098 | .60 | .42 | .48 | 8.52 | .46 | .075  | 1                                  | 149                                              | 158                  | 19.3                                            | 61.3  | 51.5                        | 51.8                                         | 47    |         |
|         |      |     |     |     |      |     |       | 4                                  | 147                                              | 160.5                | 17.9                                            | 58.5  | 53.8                        | 50.8                                         | 48.8  |         |
| B       | .100 | .26 | .31 | .48 | 7.93 | .45 | .077  | 1                                  | 146                                              | 157                  | 19.3                                            | 64.7  | 51.5                        | 51                                           | 47.5  |         |
|         |      |     |     |     |      |     |       | 4                                  | 148                                              | 162                  | 17.9                                            | 57.7  | 48.8                        | 48.5                                         | 47.3  |         |
| C       | .108 | .40 | .30 | .95 | 8.82 | .46 | .076  | 1                                  | 146                                              | 160                  | 17.9                                            | 58.5  | 48.5                        | 51                                           | 47.5  |         |
|         |      |     |     |     |      |     |       | 4                                  | 132                                              | 158                  | 17.9                                            | 59.9  | 54.5                        | 52.3                                         | 48.8  |         |
| D       | .100 | .22 | .33 | .98 | 8.67 | .48 | ----- | 1                                  | 132                                              | 146                  | 21.5                                            | 65.4  | 66.6                        | 65.5                                         | 64.5  |         |
|         |      |     |     |     |      |     |       | 4                                  | 116                                              | 145                  | 20.0                                            | 61.3  | 70.8                        | 68.3                                         | 65.5  |         |

Table 1 lists welding conditions used in preparing four of our improved weld deposits designated A, B, C and D (see

To illustrate the insensitivity of as-welded properties of our deposits to heat input, Table 3 compares data on two deposits,

E and F, prepared with 5/32-inch-diameter low-hydrogen lime-fluoride covered electrodes under conditions similar to those shown in Table 1, at respective heat inputs of 30.6 kilojoules per inch, generally considered desirably low, and 59.3 kilojoules per inch, which is rather high for 5/32-inch electrodes of the high strength type. The deposit chemical analyses were virtually identical; that for deposit E is shown at the top of the table. Although a slight drop in yield strength occurred with the higher heat input, the lower yield strength was still well above the 130 ksi minimum required of deposits of this type; tensile strength and Charpy energy absorption were only slightly affected by the higher heat input.

Heat-treated properties of our deposits are dependent on the specific heat treatment employed. We prefer to employ a standard heat treatment consisting of austenitizing at 1,500° F. for 1 hour, water quenching, tempering at 1,100° F. for one hour and water quenching again. In general an increase in tempering temperature will cause a decrease in yield and tensile strength and an increase in Charpy V-notch impact strength in the heat-treated deposit.

10 While we have described certain present preferred embodiments of the invention it is to be distinctly understood that the invention is not limited thereto but may be otherwise variously embodied within the scope of the following claims.

TABLE 4

Compositions and properties of as-welded and heat-treated deposits

| Deposit | Electrode diameter, inches | C   | Mn  | Si  | Cr   | Ni  | Mo   | V         | Condition* | Yield strength (0.2% offset), K s.i. | Elongation in 1.4 inches, percent | Red. of area, percent | Charpy V-notch energy absorption, ft.-lb. |              |              |
|---------|----------------------------|-----|-----|-----|------|-----|------|-----------|------------|--------------------------------------|-----------------------------------|-----------------------|-------------------------------------------|--------------|--------------|
|         |                            |     |     |     |      |     |      |           |            | Tensile strength                     | 80° F.                            | 0° F.                 | -60° F.                                   |              |              |
| G-----  | 5/32 .083                  | .66 | .42 | .41 | 8.30 | .52 | .082 | {AW<br>HT | 155<br>165 | 167.5<br>170                         | 17.9<br>17.9                      | 59.2<br>60.7          | 53.2<br>56.3                              | 49.8<br>48.5 | 43.8<br>41.3 |
| E-----  | 5/32 .085                  | .52 | .51 | .43 | 8.29 | .49 | .065 | {AW<br>HT | 155<br>160 | 165<br>170                           | 16.4<br>17.9                      | 59.9<br>59.2          | 47.8<br>53                                | 44.8<br>51   | 42.3<br>45   |

\*AW=As-Welded; HT=Heat-Treated.

Table 4 lists compositions, as-welded properties and heat-treated properties in 1-inch thick specimens of two of our improved deposits prepared with low hydrogen lime-fluoride covered electrodes of one-eighth inch and five thirty-seconds inch diameters respectively under conditions similar to those shown in Table 1. Deposit E is the same deposit E shown in Table 3. It will be seen from Table 4 that both as-welded and heat-treated our improved weld deposits exhibit excellent strength and toughness for both electrode sizes tested.

Graphical and statistical study of the data generated in series of experiments from which the data of Tables 2, 3 and 4 were obtained produced the above described limits of analyses of our improved weld deposits.

Although the deposits described in Tables 2, 3 and 4 were produced with low hydrogen lime-fluoride covered electrodes, 40 similar results have been achieved with deposits produced by the gas-metal arc (GMA) process; typical GMA welding involves a .062-inch diameter bare wire electrode, 320 amperes and 26 volts direct current reverse polarity and 98 per cent. argon, 2 per cent. oxygen shielding gas at 50 cubic feet per hour flow rate. Similarly, our improved weld deposits may be produced by other welding processes such as gas-tungsten-arc welding, submerged arc welding, electroslag welding, etc. Any such process should be suitable as long as the weld deposit conforms to the above described composition.

30

35

50

We claim:

1. A composite comprising a base consisting essentially of

|            | % by weight  |
|------------|--------------|
| carbon     | 0.14 maximum |
| manganese  | 0.55-0.95    |
| silicon    | 0.18-0.37    |
| chromium   | 0.36-0.74    |
| nickel     | 4.68-5.32    |
| molybdenum | 0.27-0.68    |
| vanadium   | 0.04-0.11    |
| iron       | balance      |

having thereon a weld deposit consisting essentially of

|            | % by weight |
|------------|-------------|
| carbon     | 0.03-0.12   |
| manganese  | 0.05-1      |
| silicon    | 0.2-0.7     |
| chromium   | up to 1     |
| nickel     | 6.5-11      |
| molybdenum | up to 1     |
| vanadium   | up to 0.12  |
| iron       | balance     |

which weld deposit in the heat treated condition produced by austenitizing at 1,500° F. for 1 hour, water quenching, tempering at 1,100° F. for 1 hour and water quenching exhibits a yield strength of at least 130 ksi and Charpy V-notch energy absorption at -60° F. of at least 20 ft.-lbs.

\* \* \* \* \*

55

60

65

70

75

UNITED STATES PATENT OFFICE  
CERTIFICATE OF CORRECTION

Patent No. 3,656,918 Dated April 18, 1972

Inventor(s) William T. DeLong and Paul T. Corcoran

It is certified that error appears in the above-identified patent and that said Letters Patent are hereby corrected as shown below:

In the table in the ABSTRACT, opposite "Chromium" under "Broad", "up to 1.10" should read --up to 1.0--.

Column 3, line 21, "22 B°" should be --22-1/2°--; column 5, in Table 4, after "G" and "E" under "Deposit", cancel the equal signs; line 43, ".062 - diameter" should be --.062" - diameter--; column 6, in Table 4, opposite "G" under "80° F.", "53.2" should be --53.5--.

Signed and sealed this 15th day of August 1972.

(SEAL)

Attest:

EDWARD M.FLETCHER, JR.  
Attesting Officer

ROBERT GOTTSCHALK  
Commissioner of Patents